

## UNITED STATES PATENT OFFICE

2,061,860

## METHOD OF DYEING AND PRINTING VEGETABLE AND ARTIFICIAL FIBERS

Willy Tischbein, Leverkusen-Kuppersteg, Germany, assignor to General Aniline Works, Inc., New York, N. Y., a corporation of Delaware

No Drawing. Application August 18, 1934, Serial No. 740,527. In Germany September 1, 1933

## 4 Claims. (Cl. 8—5)

The present invention relates to an improved method of dyeing and printing vegetable or artificial fibers by means of leuco sulfuric acid ester salts of vat dyestuffs.

It is known that vegetable and artificial fibers can be dyed and printed by means of leuco sulfuric acid ester salts of vat dyestuffs. The object of my present invention is an improvement as to fastness and vividness of the dyeings and prints obtained thereby. This invention is based on the discovery that excellently fast and vivid shades are obtained by impregnating the fibers, prior to the printing and dyeing by means of the leuco sulfuric acid ester salts with such organic bases or the salts thereof, as are capable of forming insoluble or at least difficultly soluble salts with the leuco sulfuric acid esters employed. It is to be understood that the subsequent dyeing and printing of the fibers thus impregnated is performed according to the methods usually applied in the art.

I wish to point out that the present invention contemplates the employment of the bases of the character described generally, it being understood that according to my experiments every organic base, which forms insoluble or at least difficultly soluble salts with the leuco sulfuric acid esters employed, is capable of accomplishing the desired result, regardless as to whether it shows affinity to the fiber or not.

Obviously, the choice of the bases to be employed depends on the above described characteristics only and, this doctrine being given, everyone skilled in the art can ascertain by simple experiments, whether the bases intended are suitable for the purpose in question.

As examples of bases which have proved to be excellently suitable for this purpose there may be mentioned, for instance, amines, ammonium- and phosphonium bases, such as the condensation products of chlorinated paraffines with ammonia, cyclohexylmethyldiethylammonium iodide, dimethyltetrahydroquinolinium iodide, trimethylammoniummethylsulfate of mono-oleylethylidiamine or of monostearyl-para-phenylene diamine, mixtures of higher polyethylene polyamines, octadecylpyridinium bromide, triphenylbenzylphosphonium chloride, triphenyldichlorobenzylphosphonium chloride. It is pointed out that the compounds enumerated above yield insoluble or at least difficultly soluble salts with the leuco sulfuric acid esters, the term "at least difficultly soluble salts" used in the appended claims being intended to embrace both difficultly soluble and insoluble salts.

The effect obtained by my present invention is

illustrated by the following arguments: It is known that many leuco sulfuric acid esters of vat dyestuffs show an insufficient affinity for vegetable and artificial fibers and are, on the other hand, insufficiently soluble for being employed in concentrated aqueous solution. For instance, if employing in the skein-dyeing a proportion of dye liquor of at least 1:15-1:20, only a minor part of the dyestuff is fixed to the fiber, whereas, on the other hand, the danger of salting out is involved. This disadvantage is completely overcome by treating the fibers by means of the bases of the character described prior to the printing or dyeing as described above. It follows therefrom that the present invention rendered it technically possible for the first time to employ leuco sulfuric acid esters of vat dyestuffs generally in the usual dyeing apparatus. The same holds true with regard to the dyeing of piece goods as up to the present time leuco sulfuric acid esters could only be employed for dyeings of light shades. Similar remarks apply to the printing of vegetable or artificial fibers, it being understood that the subsequent development of the prints can be effected according to usual methods, for instance, according to the nitrite-process with or without steaming.

The following examples will illustrate the invention, without, however, restricting it there-

30

to:—

## Example 1

50-100 grams of cotton yarn, bleached or raw, are treated with an aqueous solution of 35° C. containing 6 grams of the condensation product of trichlorinated paraffine and a mixture of polyethylene polyamines (obtainable by the action of NH<sub>3</sub> on ethylene chloride), squeezed and dried. The cotton yarn thus treated is then dyed for half an hour at a temperature falling from 40°-30° C. in a bath containing per litre 3.5 grams of the alkali salt of the acid sulfuric acid ester of the leuco compound of 6,6'-diethoxy-2,2'-bisthionaphthene indigo, 10 grams of sodium nitrite and 35 grams of sodium sulfate (proportion of the dye liquor 1:10-1:20), squeezed off, immediately oxidized for a short time in hot water of 75° C. which contains per litre 35 ccs. of sulfuric acid (66° Bé.) and thoroughly rinsed. Thereupon it is neutralized and soaped while boiling. The dyeing thus obtained shows a considerably deeper shade than a dyeing obtained in the absence of the above mentioned condensation product.

The same effect can be observed if applying

45

50

55

the salts of other sulfuric acid ester of the leuco compounds of vat dyestuffs, such as for example, Bz-2-Bz-2' - dimethoxydibenzanthrone, 5.7'-dibromo-2'-indole-2-anthracene indigo, benzoquinone-di-para-chloranilide, 4-methyl-6-chloro-6'-methoxy-thioindigo, the dyestuff obtained according to U. S. P. 1,782,706, 2.1-naphthioindigo and the like.

When using the above mentioned base for impregnating cotton yarn in a weakly acid bath (6 grams of base and 2-15 ccs. of acetic acid per litre) and employing the same dyeing method, a similar deepening of shades is obtained; as dyestuffs there may be used the alkali salts of the acid sulfuric acid esters of the leuco compounds of vat dyestuffs, such as for example, 4.4'-dimethyl-6.6'-dichloro-bis-thionaphthene indigo, 2.1-naphthioindigo, 6.6'-diethoxy-2.2'-bisthionaphthene indigo, dimethyl-trichloro thioindigo etc. A still stronger deepening of the shades is obtained, if the base in question is applied on the fibre in a larger amount by salting out and the dyeing is performed in the usual manner with the ester dyestuffs mentioned.

Example 2

50-100 grams of cotton yarn or fabrics, which have been impregnated with a solution of 5 grams of triphenyldichlorobenzylphosphonium chloride in one litre of water at a temperature of about 35° C. for half an hour, show, when dyed in accordance with the method described in Example 1 with the alkali salts of the acid sulfuric acid esters of the leuco compounds of 4.4'-dimethyl-6.6'-dichloro-bis-thionaphthene indigo, the dyestuff of the following formula



obtainable according to the U. S. Patent 1,782,706 or of benzoquinone-di-para-chloranilide far deeper shades than dyeings obtained on untreated cotton.

Similarly improved dyeings may also be obtained by pretreating 50-100 grams of cotton yarn or fabrics with 1 litre of an aqueous solution containing 4 grams of the base described in Example 1 and 2 grams of triphenyldichlorobenzyl-phosphonium chloride at a temperature of 35° C. for half an hour and printing the same according to usual methods with the alkali salts of the acid sulfuric acid ester of the leuco compounds of vat dyestuffs, such as for example, of benzoquinone-di-para-chloranilide, 6.6'-diethoxy-2.2'-bisthio-naphthene indigo, 2.1-naphthioindigo and 4'-methyl-6-chloro-6'-methoxy-thioindigo.

Example 3

50-100 grams of cotton yarn or fabrics yield also shades of improved deepening when pretreated with 1 litre of an aqueous solution containing 3-5 grams of octadecylpyridinium bromide for half an hour at 35° C. and dyed with the alkali salts of acid sulfuric acid esters of the leuco compounds of vat dyestuffs, such as, for example, 6.6'-diethoxy-2.2'-bisthio-naphthene indigo or 4-methyl-6-chloro-6'-methoxy-thioindigo. Similar effects are obtained by dyeing the acid sulfuric acid esters of the leuco com-

pounds of vat dyestuffs on cotton yarn, which has been impregnated according to the method described above with the condensation products of halogenated paraffines and ammonia or with cyclo-hexylmethyl-diethylammonium iodide, dimethyltetrahydro-quinaldinium iodide, mixtures of higher polyethylene polyamines (see Example 1), triphenylbenzylphosphonium - chloride, trimethylammoniummethylsulfate of monooleyl-ethylene diamine or monostearyl-para-phenylene diamine.

Example 4

Artificial silk yarn or fabrics (for example, viscose silk) are treated with the bases obtainable by the reaction of trichlorinated paraffine with polyethylene polyamines, alone or together with triphenyldichlorobenzyl phosphonium chloride, or alone with the latter product, in a neutral, acid or alkaline bath for half an hour at 35° C. (proportion of the dye liquor 1:10-1:20), and then dyed with the alkali salts of the acid sulfuric acid esters of the leuco compounds of benzoquinone-di-para-chloroanilide, 4-methyl-6-chloro-6'-methoxy-thioindigo, 6.6'-diethoxy-2.2'-bis-thionaphthene indigo or similar vat dyestuffs.

The dyeings obtained show an improved depth of color compared with corresponding dyeings on unpretreated artificial silk.

Example 5

Cotton and artificial silk material or also mixed fabrics which have been pretreated in a neutral, acid or alkaline bath with bases obtained from ammonia or amines and trichlorinated paraffines as described above, yield on printing with the alkali salts of the acid sulfuric acid esters of the leuco compounds of vat dyestuffs, deeper prints than they can be obtained on unpretreated fabrics.

Example 6

50-100 grams of bleached or raw cotton yarn or artificial silk are treated for 20-25 minutes in an aqueous neutral, acid or alkaline solution of 35° C. containing 2-6 grams per litre of a product obtainable by condensation of polyethylene polyamine and cyanuric chloride and subsequent peralkylation by means of dimethylsulfate, squeezed off and dried, though drying is not absolutely necessary. The material thus treated is then introduced into a bath containing 3.5 grams of the alkali salt of the acid sulfuric acid ester of the leuco compound of 6.6'-diethoxy-2.2'-bisthionaphthene indigo, 10 grams of sodium nitrite and 35 grams of sodium sulfate per litre for half an hour at raising or from 40° to 30° C. falling temperature; thereupon it is thoroughly rinsed, neutralized and soaped at the boil. A very strong deepening of the shade is obtained thereby.

The same effect results when treating the material described above with the alkali salts of the acid sulfuric acid esters of the leuco compounds of vat dyestuffs, such as Bz-2-Bz-2'-dimethoxy-dibenzanthrone, benzoquinone-di-para-chloroanilide, methylchloromethoxy thioindigo, 2.1-naphthioindigo and the like, in corresponding amounts. The above described product of the condensation of polyethylene polyamine and cyanuric chloride can be prepared by dissolving 18.5 parts of cyanuric chloride in about 200 parts of trichloroethylene, adding thereto a solution of 40.5 parts of a polyethylene polyamine mixture of a boiling point of between 90° C. and 75

350° C. at 15 mm. pressure in 80 parts of a ten fold normal hydrochloric acid, stirring for some time at 20° to 25° C., adding thereto a concentrated solution of 160 parts of sodium acetate and thereupon neutralizing the acid by gradually adding an aqueous solution of 58 parts of sodium carbonate. The solvent is then removed by water distillation, the remaining solution is concentrated and the condensation product crystallizes therefrom upon cooling.

10 **Example 7**

50-100 grams of bleached or raw cotton yarn or artificial silk or mixtures of these materials are treated for 20-25 minutes in an aqueous, 15 neutral, acid or alkaline solution of 35° C. containing 2-6 grams per litre of heptadecylamine acetate, squeezed off and dried. Working up is performed as described in Example 6. A very 20 strong deepening of color is obtained.

25 **Example 8**

50-100 grams of bleached or raw cotton yarn or artificial silk or mixtures of these materials 25 are treated for 20-25 minutes in an aqueous, neutral, acid or alkaline solution of 35° C. containing per litre 2-6 grams of heptadecylamine peralkylated with dimethylsulfate, squeezed off, dried and further worked up as described in 30 Example 6.

A similar effect as to the depth of color is obtained by the same process with the exception that the condensation products obtainable by causing a primary or secondary aliphatic amine 35 containing at least one hydrocarbon radicle with more than 8 carbon atoms or a mixture thereof to react with a halogen-alkylamine which is disubstituted on the nitrogen atom by alkyl groups are used instead of the peralkylated 40 heptadecylamine.

30 **Example 9**

50-100 grams of bleached or raw cotton yarn

or artificial silk or a mixture of these materials are treated for 20-25 minutes in 1 litre of an aqueous alkaline solution of 35° C., containing 2-6 grams of the reaction product of ethylene oxide on a mixture of polyethylene polyamines 5 (obtainable according to the method described in Example 1), squeezed off, dried if necessary, and worked up as described in Example 6. Strong deepened shades are obtained by this process.

10 I claim:—

1. In the process of dyeing and printing vegetable and artificial fibers by means of leuco sulfuric acid ester salts of vat dyestuffs the improvement which consists in impregnating the fibers 15 prior to the action of the leuco sulfuric acid ester salts with organic bases selected from the group consisting of high molecular aliphatic nitrogen bases and quaternary ammonium and phosphonium bases and the salts thereof.

2. In the process of dyeing and printing vegetable and artificial fibers by means of leuco sulfuric acid ester salts of vat dyestuffs, the improvement which consists in impregnating the fibers prior to the action of the leuco sulfuric 25 acid ester salts with a condensation product of a trichlorinated paraffine and a mixture of polyethylene polyamines.

3. In the process of dyeing and printing vegetable and artificial fibers by means of leuco sulfuric acid ester salts of vat dyestuffs, the improvement which consists in impregnating the fibers prior to the action of the leuco sulfuric acid ester salts with a peralkylated heptadecylamine.

4. In the process of dyeing and printing vegetable and artificial fibers by means of leuco sulfuric acid ester salts of vat dyestuffs, the improvement which consists in impregnating the fibers prior to the action of the leuco sulfuric acid ester salts with heptadecylamine acetate.

30 35 40  
WILLY TISCHBEIN.